

Mar. 20, 1923.

1,449,053.

C. PACK.

METHOD OF MAKING DIE CASTINGS.

FILED NOV. 15, 1921.

*Fig. 1,*



*Fig. 3,*



*Fig. 2,*



*Fig. 4,*



*Fig. 5.*



INVENTOR

BY *Charles Pack*  
*J. Edwards* ATTORNEY

Patented Mar. 20, 1923.

1,449,053

# UNITED STATES PATENT OFFICE.

CHARLES PACK, OF NEW YORK, N. Y., ASSIGNOR TO DOEHLER DIE CASTING COMPANY,  
OF BROOKLYN, NEW YORK, A CORPORATION OF NEW YORK.

## METHOD OF MAKING DIE CASTINGS.

Application filed November 15, 1921. Serial No. 515,213.

To all whom it may concern:

Be it known that I, CHARLES PACK, a citizen of the United States, residing in the borough and county of Queens, city and 5 State of New York, have invented certain new and useful Improvements in Methods of Making Die Castings, of which the following is a specification.

This invention relates to the art of die 10 casting, and more particularly to a method for producing die castings.

It is well known that the structure of a die casting is relatively dense on the chilled surfaces, and that the structure is less dense 15 and more porous as the interior of the casting is approached. In heavy sections blow holes of varying sizes will be found toward and in the center of the casting. When the casting does not require machining this is 20 not objectionable, but when the casting must be machined, these blow holes are very objectionable, since they are apt to be uncovered in the machining operation. The object of my invention is to provide a method 25 for producing die castings whereby predetermined portions of the die casting will be free from blow holes, and a method of producing a die casting which may be machined interiorly without uncovering blow 30 holes. Further objects of my invention include the method of creating an area of unusually great density at interior portions of a die casting, and a method of forming an internally located chilled surface in a die 35 casting. Other objects will be in part obvious and in part pointed out hereafter.

In accordance with my invention, I provide a core of machinable material approximately the size and shape of the cut which 40 it is desired to form in the finished casting, the core being preferably somewhat smaller than the cut in size. I then form a die casting about this core, and after the casting has become set, remove the core together with 45 a slight portion of the casting by a machining operation to form the desired finished casting.

In order that a clearer understanding of 50 my invention may be had, attention is hereby directed to the accompanying drawings forming a part of this application and illustrating certain possible embodiments of my invention. Referring to the drawings, Figure 1 is a section of a casting showing the core in place; Figure 2 is a view similar

to Figure 1 showing the finished casting after the desired cut has been formed therein; Figure 3 is a top view of the casting illustrated in Figure 1 having a portion broken away for the sake of clearness; Figure 4 is a sectional view of another casting showing the core in place; and Figure 5 is a sectional view similar to Figure 4 showing the finished casting with the desired cut formed therein.

My improved method may be applied to the production of die castings irrespective of their shape or size and to the production of cuts in die castings extending into any surface thereof. In Figures 1, 2 and 3 of the 70 drawings I have illustrated the application of my invention to the production of a die cast ring having an undercut annular groove formed to extend inwardly from the inner surface of the ring. In carrying out my 75 method I first provide an annular ring 1 of machinable material having an annular portion 2 approximately the same size and shape of the undercut which it is desired to form in the finished casting. Using this 80 core 1 as an insert I form a die casting 3 thereabout, and after the casting has become set, I remove the core 2 by a machining operation and thus provide the desired 85 undercut in the casting 3. By casting the 90 ring 3 about the core 1 the surfaces 4, which contact the core 1, become chilled and the portions of casting 3 adjacent these surfaces are relatively dense and free from blow holes, so that the casting may be machined 95 for a distance inwardly of these surfaces without the danger of uncovering or exposing blow holes. I preferably make the core 1 slightly smaller in size than the size of the desired undercut, so that the machining operation may be continued to some extent into the core 3 to form the desired undercut and to place a machine finish on the surfaces of the undercut. In casting a ring as 100 illustrated in Figures 1, 2 and 3 of the drawings the insert or core 1, if desired, may have a portion 5 extending outwardly to aid in positioning the core in the desired position in the die, it being understood that such portion 5 is to be removed by machining 105 or other operation if such insert is not desired in the finished casting.

In Figures 4 and 5 I have illustrated my method as applied in the casting of a hollow cylindrical die casting having a plural- 110

ity of annular grooves cut on the interior thereof, the grooves being of various depths and widths. To form the casting here illustrated I first provide a core or insert 6 of a 5 diameter approximately equaling the smallest interior diameter of the finished casting, and of a length approximately the axial distance covered by the undercuts. I form a die casting 7 about the core 6, the casting 7, 10 as shown, having annular end flanges 8 and 9 overlapping the outer ends of the core 6. In forming the casting 7 about the core 6 in the manner above described, it will be noted that the casting will have interiorly located 15 chilled surfaces 10 where the casting abuts against the outer circumference of the core 6. The structure of the die casting 7 adjacent the surfaces will be relatively dense and solid and free from blow holes, and the desired grooves 11, 12 and 13 respectively, may 20 be machined in the die casting without the danger of exposing blow holes. The core may be entirely machined away, and then the grooves 11, 12 and 13 formed in the 25 casting 7 by continuing the machining operation.

In producing castings by the above method in quantities, I preferably employ a die adapted to form not only the casting about 30 the inserted core, but is also adapted at the same operation to form a core which may be used in the production of the next succeeding casting. In this way the cost of producing the necessary cores by separate operations is eliminated. For instance, in producing a quantity of castings of the type 35 illustrated in Figures 1, 2 and 3, the die may be fashioned to contain a cavity for casting the ring 3 about an inserted core 1 and another cavity wherein a core 1 may be die cast. When the casting has been made the 40 newly cast core 1 may be broken off from the casting 3 at the gate. The newly cast core 1 is then used as an insert in the next 45 casting operation.

It is to be understood that my invention

relates to the forming of dense portions of chilled surfaces in any part of a die casting, and to the forming of cuts on the outside of a casting as well as on the inside. 50

As many changes could be made in carrying out the above method without departing from the scope of the invention, it is intended that all matter contained in the above description shall be interpreted as illustrative and not in a limiting sense. 55

What I claim is:—

1. A method of producing a die casting, which comprises, providing a core of machinable material, forming a die casting 60 about said core and machining the core away from said casting.

2. A method of producing a die casting having a cut, which comprises, providing a core of machinable material approximately 65 the size and shape of the desired cut, forming a die casting about said core and machining away said core from said casting.

3. A method of producing a die casting having a cut, which comprises, providing a 70 core of machinable material slightly smaller in size than the desired cut and approximating the cut in shape, forming a die casting about said core and machining away said core and a portion of the casting adjacent 75 thereto to form the cut.

4. A method of producing a plurality of die castings, which comprises, successively forming die castings, each comprising a casting formed about an insert and an integral casting constituting a replication of 80 said insert, severing the newly-formed insert from the other casting, and using said newly-formed insert as an insert in forming a succeeding die casting. 85

This specification signed and witnessed this 4th day of November, 1921.

CHARLES PACK.

Witnesses:

WILLIAM R. AHRBERG,  
WILLIAM E. BAUERSCHMIDT.